

# United States Patent [19]

Inagaki

[11] Patent Number: 4,550,243

[45] Date of Patent: Oct. 29, 1985

## [54] HEAT ROLLER FIXING DEVICE

[75] Inventor: Sanji Inagaki, Toyokawa, Japan

[73] Assignee: Minolta Camera Kabushiki Kaisha, Osaka, Japan

[21] Appl. No.: 545,492

[22] Filed: Oct. 26, 1983

## [30] Foreign Application Priority Data

Nov. 4, 1982 [JP] Japan ..... 57-194218

[51] Int. Cl.<sup>4</sup> ..... G03G 15/20

[52] U.S. Cl. ..... 219/216; 219/469; 355/3 FU; 432/60

[58] Field of Search ..... 219/216, 469, 470, 471, 219/388; 432/60, 59, 227, 228; 355/3 FU

## [56] References Cited

### U.S. PATENT DOCUMENTS

- |           |         |           |          |
|-----------|---------|-----------|----------|
| 3,235,772 | 2/1966  | Gurin     | 219/216  |
| 4,179,601 | 12/1979 | Tarumi    | 219/469  |
| 4,257,699 | 3/1981  | Lentz     | 219/216  |
| 4,272,179 | 6/1981  | Seanor    | 355/3 FU |
| 4,320,714 | 3/1982  | Shimazaki | 432/60   |
| 4,372,246 | 2/1983  | Azar      | 219/216  |
| 4,434,355 | 2/1984  | Inagaki   | 219/469  |

## OTHER PUBLICATIONS

Evans, H. E. and A. A. Parker, "Hot Roll Fuser", IBM Tech. Disc. Bull., vol. 25, No. 7B, Dec. 1982, p. 3985.

Primary Examiner—C. L. Albritton

Assistant Examiner—Teresa J. Walberg

Attorney, Agent, or Firm—Wenderoth, Lind & Ponack

## [57] ABSTRACT

A heat roller fixing device for use in an electrophotographic copying apparatus and the like, which includes a heating roller constituted by a fluorine resin layer laminated on an electrically conductive core member through a primer layer, the heated roller being driven for rotation, and a pressure roller constituted by an electrically insulative layer on another electrically conductive core member and held in contact with the heating roller for simultaneous rotation with the heating roller so as to fix a charged toner image formed on copy paper onto the copy paper by causing the copy paper carrying the toner image thereon to pass between the heating roller and pressure roller. The primer layer is composed of a primer having incorporated therein an electrically conductive material, and the primer of the primer layer is partly exposed at the surface of the fluorine resin layer. Triboelectric charges produced on the surface of the fluorine resin layer are released by grounding through the primer layer and the electrically conductive core member.

14 Claims, 20 Drawing Figures



FIG. I



FIG.2



FIG. 3



FIG.4



FIG.5



FIG. 6



FIG.7



FIG. 8



FIG.9



FIG.10



FIG.11



FIG.12



FIG.13



FIG.14



FIG. 15



FIG. 16



FIG.17



FIG.18



FIG.19



| Example                |                       |     | Offset property with respect to positively charged toner in check point paper pass. time 2-5 min. |    |                    | Offset property with respect to negatively charged toner in check point paper pass. time 60 min. |     |    |     |    |     |    |
|------------------------|-----------------------|-----|---------------------------------------------------------------------------------------------------|----|--------------------|--------------------------------------------------------------------------------------------------|-----|----|-----|----|-----|----|
|                        |                       |     | Fixing temp. (°C)                                                                                 |    |                    | Fixing temp. (°C)                                                                                |     |    |     |    |     |    |
| Thickness of layer (μ) | 4th layer (PFA resin) |     | 2nd layer (PFA resin)                                                                             |    | 1st layer (primer) |                                                                                                  | 130 |    | 170 |    | 210 |    |
|                        | 0                     | 6   | 30~40                                                                                             | -  | 15                 | 15                                                                                               | 15  | 15 | 15  | 15 | 15  | 15 |
|                        | Comparative Example   | 1.0 | 5                                                                                                 | 15 | 15                 | 15                                                                                               | 15  | 15 | 15  | 15 | 15  | 15 |
| Example 1              | 0.5                   | 5   | 15                                                                                                | 15 | 15                 | 15                                                                                               | 15  | 15 | 15  | 15 | 15  | 15 |
| Example 2              | 1.5                   | 5   | 15                                                                                                | 15 | 15                 | 15                                                                                               | 15  | 15 | 15  | 15 | 15  | 15 |
| Example 3              | 2.0                   | 5   | 15                                                                                                | 15 | 15                 | 15                                                                                               | 15  | 15 | 15  | 15 | 15  | 15 |
| Example 4              | 1.0                   | 5   | 15                                                                                                | 15 | 23                 | 30                                                                                               | 30  | 30 | 30  | 30 | 30  | 30 |
| Example 5              | 1.5                   | 15  | 35                                                                                                | -  | -                  | -                                                                                                | -   | -  | -   | -  | -   | -  |

Carbon black add amount in primer(part by wt)

FIG.20

## HEAT ROLLER FIXING DEVICE

## BACKGROUND OF THE INVENTION

The present invention relates to a heat roller fixing device, and more particularly to a heat roller fixing device which, as shown in FIG. 1, comprises a heating roller 5 incorporating a heater 4 and having a fluorine resin layer 3 over an electrically conductive core member 1 with a primer layer 2 interposed therebetween, and a pressure roller 8 having an insulating layer 7 over an electrically conductive core member 6 and adapted for pressing contact with the heating roller 5. When the fixing device is in operation, the heating roller 5 is heated by the heater 4 at a suitable temperature of 140° to 180° C. in accordance with the kind of toner used. Copy paper P having a charged toner image 9 formed thereon is passed between the rollers 5 and 8 with the image bearing surface facing the heating roller 5, whereby the toner image 9 is fixed onto the copy paper P. The drawing further shows a guide plate 10, a discharge roller 11, a separating pawl 12 and a thermistor 13.

With heat roller fixing devices of this type, the surface of the heating roller has good release properties sufficient to prevent thermal adhesion of the toner without necessitating application of silicone oil or like offset preventing agent, or with use of only a very small amount of such agent. The device therefore renders the copy paper free from stains and gives prints which feel good to the touch. However, the fluorine resin surface layer 3 of the heating roller 5, which is triboelectrically charged by the insulating surface layer 7 of the pressure roller 8 or by the copy paper P, is liable to electrostatically attract toner images and to permit offset, whereby the offset preventing agent is unable to preclude the offset due to triboelectrification.

The present inventor, together with other inventors, has already provided a heat roller fixing device wherein the primer layer 2 of the heating roller 5 is formed of a fluorine resin containing carbon black and which is adapted to prevent the offset due to such triboelectrification (U.S. patent application Ser. No. 351,930 filed on Feb. 24, 1982). This device solved a problem conventionally experienced. With the known device shown in FIG. 1, the triboelectric charges on the heating roller 5, which were of negative polarity when the assembly started passage of paper, reached a maximum of more than -600 V upon lapse of about 5 minutes, then reversed to positive polarity upon lapse of about 10 minutes and thereafter reached about +200 V max. as illustrated in FIG. 9 by hatching, whereas negative charging is almost avoidable with the device of Serial No. 351,930. Accordingly the heating roller 5 is readily held at positive polarity to inhibit the electrostatic attraction of toner to the roller 5 and prevent offset when the toner is charged positively.

Nevertheless, since it is nearly impossible to eliminate the positive charges, offset is unavoidable when a toner of negative polarity is used, so that the device is limited in the polarity of the toner to be used, since the charges could produce an adverse effect.

## SUMMARY OF THE INVENTION

An object of the present invention is to provide a heat roller fixing device wherein negative and positive triboelectrification of the heating roller is inhibited to pre-

vent the offset of either positively charged toner or negatively charged toner.

The present inventor has found that the above object can be fulfilled by making use of the electrical conductivity of the aforementioned carbon black-containing primer layer, i.e., by partly exposing the primer layer at the surface of the fluorine resin layer to release triboelectric charges by grounding through the primer layer and the electrically conductive core member.

More specifically, the present invention provides a heat roller fixing device of the type shown in FIG. 1 wherein a primer having incorporated therein an electrically conductive material is used for the primer layer of the heating roller, the fixing device being characterized in that the heating roller comprises at least one primer layer and at least one fluorine resin layer formed over the primer layer to provide the surface of the heating roller, the primer layer being partly exposed at the surface of the fluorine resin layer.

Because of this structure, the surface of the heating roller has improved strength, is less susceptible to defacement due to contact with the separating pawl or thermistor, possesses high durability, is low in potential when triboelectrically charged positively or negatively, and will not produce an adverse effect on other members or other process.

## BRIEF DESCRIPTION OF THE DRAWINGS

FIG. 1 is a side elevation in section showing a conventional heat roller fixing device which is generally used and to which the present invention is applied;

FIGS. 2 to 7 are fragmentary enlarged views illustrating a process for preparing a heating roller of the present invention;

FIG. 2 shows the step of coating an electrically conductive core member with a primer;

FIG. 3 shows the step of electrostatically coating the resulting primer coating with a finely divided fluorine resin;

FIG. 4 shows the step of forming a second primer coating;

FIG. 5 shows the step of forming a second finely divided fluorine resin coating electrostatically;

FIG. 6 shows the step of baking the resulting overall coating in an oven;

FIG. 7 shows a grinding step for exposing all penetrating portions of the primer at the outer peripheral surface of the roller;

FIG. 8 is a cross sectional view showing the heating roller prepared according to the present invention;

FIGS. 9 to 19 are diagrams showing the charging characteristics of the heating rollers prepared in a comparative example and examples of the present invention; and

FIG. 20 is a diagram showing the offset properties of the heating rollers of the comparative example and the examples of the present invention as determined during the period of 2 to 5 minutes after the start of passage of copy paper and also as determined 60 minutes after the start of passage of paper.

## DETAILED DESCRIPTION OF THE INVENTION

The present invention provides a heat roller fixing device of the type shown in FIG. 1 wherein a primer having incorporated therein an electrically conductive material is used for the primer layer 2 of the heating roller 5. The device is characterized in that the heating

roller 5 comprises at least one primer layer 2 and at least one fluorine resin layer 3 which is formed over the primer layer 2 to provide the surface of the heating roller 5, and in that the primer layer 2 is partly exposed at the surface of the fluorine resin layer 3.

Examples of materials useful for the electrically conductive core member are aluminum, aluminum alloy, iron alloys such as stainless steel, and other metals.

For the fluorine resin layer, it is preferable to employ fluorine resins superior in heat resistance, such as polytetrafluoro ethylene resin (PTFE) represented by the formula



polytetrafluoro ethylene perfluoro alkoxy ethylene copolymer resin (PFA resin) represented by the formula



and the like.

The primer layer of the heating roller is formed from a primer of the solution type composed chiefly of fluorine resin, which is commercially available as an adhesive priming agent for iron alloys, aluminum alloys and like metal materials mentioned. Examples of useful primers are COOKWEAR A PRIMER WHITE 459-882 (brand name, product of Du Pont Co., Ltd. Japan), MP902BN (brand name, product of Mitsui Phlorochemical Co., Japan), etc. Useful as the electrically conductive material to be incorporated into the primer is a metallic powder, or carbon black which may be any of furnace black, channel black and thermal black. Examples of such products commercially available are KETCHEN BLACK EC (brand name, product of Lion Yushi Co., Ltd., Japan), SPECIAL BLACK 4 (brand name, product of Degussa Co., Ltd. Japan), CARBON BLACK MA-100 and MA-8 (brand names, products of Mitsubishi Chemical Industries Ltd., Japan), ACETYLENE BLACK (brand name, product of Denki Kagaku Kogyo Kabushiki Kaisha, Japan), etc.

The carbon black is incorporated in the primer in an amount of 0.4 to 3.0% by weight, preferably 0.5 to 2.0% by weight. If the amount is less than 0.4% by weight, the contemplated effect will not result, whereas more than 3.0% by weight of carbon black, if used, renders the primer coating composition too viscous, so as to produce irregularities in the coating and plug up the spray nozzle, making it difficult to obtain a uniform coating and to fabricate a satisfactory roller. Furthermore, an increase in the amount of carbon black entails a reduction in release properties, so that the amount is preferably smaller insofar as triboelectrification can be inhibited to prevent offset.

The insulating layer of the pressure roller is formed from an insulating material, such as natural rubber or

synthetic rubber, having rubber-like elasticity, or usually employed in producing pressure rollers.

The following process is used for preparing the heating roller which comprises at least one primer layer and 5 at least one fluorine resin layer over the primer layer, with the primer layer partly exposed at the surface of the fluorine resin layer. First, a liquid primer 2a having incorporated therein an electrically conductive material is sprayed over the surface of the electrically conductive core member 1 as shown in FIG. 2. Next, as shown in FIG. 3, a finely divided fluorine resin 3a is applied to the surface of the primer coating 2a by electrostatic powder coating before the primer 2a dries. The resulting coating is further similarly coated with the primer 10 2a and then with the fluorine resin 3a as seen in FIGS. 15 4 and 5. The primer coatings 2a and the fluorine resin coatings 3a are thereafter baked in an oven to obtain primer layers 2 and fluorine resin layers 3 in the form of a laminate as shown in FIG. 6.

20 In the baking step, the finely divided fluorine resin 3a is baked into layers 3 while permitting the primer 2a to penetrate into the layers 3 among the particles of the resin 3a, with the result that penetrating portions 2b partially extending from the primer layers 2 are formed 25 in the fluorine resin layers 3 as very well dispersed therein and are shown in FIG. 6. In the fluorine resin layer 3 sandwiched between the two primer layers 2, the penetrating portions 2b from the primer layers 2 are continuous. In the fluorine resin surface layer 3, almost 30 all the penetrating portions 2b from the primer layer 2 therebeneath are formed without reaching the surface of the fluorine resin layer 3.

Accordingly the surface of the fluorine resin surface layer 3 is ground to expose the penetrating portions 2b from the underlying primer layer 2 at the surface of the fluorine resin surface layer 3 as seen in FIG. 7.

The above process gives the heating roller 5 of FIG. 8 which comprises primer layers 2 formed of a primer 2a incorporating an electrically conductive material 35 therein and fluorine resin layers 3. The layers 2 and the layers 3 are formed alternately one over the other so as to form the surface of the heating roller 5 by one of the fluorine resin layers 3, with the penetrating portions 2b of the primer layer 2 exposed at the surface of the fluorine resin surface layer 3 as distributed over the surface. Since the heating roller 5 has the fluorine resin layer 3 over its surface, the fusion or thermal adhesion of toner 40 can be prevented. The surface portions of the fluorine resin surface layer 3 are electrically connected to the electrically conductive core member 1 by the primer layers 2 of primer 2a incorporating the conductive material and by the penetrating portions 2b thereof and are grounded via the core member 1, so that the triboelectrification of the fluorine surface layer 3 due to the frictional contact thereof with the pressure roller 8 or 45 copy paper P can be greatly inhibited irrespective of the polarity. Thus copies can be produced without offset at all times from the initial stage of operation of the fixing device irrespective of whether the toner is charge positively or negatively.

#### EXAMPLE 1

A liquid primer (MP902BN, product of Mitsui Phlorochemical Co., Japan) having a solids content of 19% by weight and containing carbon black (KETCHEN BLACK EC, product of Lion Yushi Co., Ltd., Japan) as an electrically conductive material was sprayed onto an aluminum roller serving as the electri-

cally conductive core member 1. Next, finely divided PFA resin was applied to the primer coating 2a by electrostatic powder coating before the coating dried. The resulting coating was coated similarly with primer 2a by spraying and then with finely divided PFA resin electrostatically. The overall coating was thereafter baked at about 400° C. in an oven. The outer peripheral surface of the PFA resin surface layer was subsequently ground to expose the penetrating portions from the underlying primer layer at the surface of the PFA resin surface layer, whereby a heating roller was prepared.

Table 1 shows the amount of carbon black used (per 100 parts by weight of the primer containing 19% by weight of solids), the thickness of the primer layers 2 and the PFA resin layers 3 and the amount of grinding.

The surface of another aluminum roller was covered with a commercial silicone rubber to prepare a pressure roller. A heat roller fixing device of the type shown in FIG. 1 was fabricated with use of the rollers.

TABLE 1

| Example | Amount of carbon in primer (part by wt.) | Thickness of layer ( $\mu$ ) |                       |                    |                       |                    |
|---------|------------------------------------------|------------------------------|-----------------------|--------------------|-----------------------|--------------------|
|         |                                          | 1st layer (primer)           | 2nd layer (PFA resin) | 3rd layer (primer) | 4th layer (PFA resin) | Amount of grinding |
| 1       | 1.0                                      | 5                            | 15                    | 5                  | 15                    | 5                  |
| 2       | 0.5                                      | 5                            | 15                    | 5                  | 15                    | 5                  |
|         | 1.5                                      | "                            | "                     | "                  | "                     | "                  |
|         | 2.0                                      | "                            | "                     | "                  | "                     | "                  |
| 3       | 1.0                                      | 5                            | 5                     | 5                  | —                     | 5                  |
|         | "                                        | "                            | 15                    | "                  | —                     | "                  |
|         | "                                        | "                            | 30                    | "                  | —                     | "                  |
| 4       | 1.0                                      | 5                            | 15                    | 5                  | 23                    | 5                  |
|         | "                                        | "                            | "                     | "                  | 30                    | "                  |
| 5       | 1.5                                      | 15                           | 35                    | —                  | —                     | 5                  |

The fact that the above device fulfills the object of the invention will be described with reference to the following measurements and comparative example.

#### A. Determination of charging characteristics of heating roller

The charging characteristics of the heating roller were determined during a copying operation at a temperature of 170° C. which was selected from the fixing temperature range of 140° to 180° C. for various kinds of toners. For this purpose, sheets of copy paper of A4 size bearing no toner images were passed between the two rollers at a speed of 11 cm/sec., and the maximum and minimum surface potential on the circumference of the heating roller were measured by a vibrating-type surface potentiometer. FIG. 10 shows the results.

#### B. Determination of offset properties

FIG. 9, showing the charging characteristics of the conventional heating roller to be given as the comparative example, indicates that the roller is most susceptible to the offset of positively charged toner during the period of 2 to 5 minutes after the start of passage of copy paper, and to the offset of negatively charged toner 60 minutes after the start of passage. The heating rollers prepared in the examples to follow were tested during the above period and at the above point of time at temperatures of about 120° to about 220° C. for marked offset, slight offset and non-offset to determine the temperature ranges permitting these offset phenomena, using sheets of copy paper bearing a positively charged toner image (toner: composed chiefly of styrene-acrylic resin, having a mean particle size of 14 $\mu$  and charged to 10 to 12  $\mu$ C/g) formed by electropho-

tography, and sheets of copy paper bearing a negatively charged toner image (toner: composed chiefly of styrene-acrylic resin, having a mean particle size of 14 $\mu$  and charged to 10 to 12  $\mu$ C/g) similarly formed. The results are shown in FIG. 20, in which the area hatched by oblique lines represents marked offset, the area marked with horizontal lines indicates slight offset, and the blank area shows non-offset.

#### COMPARATIVE EXAMPLE

A heat roller fixing device of the type shown in FIG. 1 was fabricated in the same manner as in Example 1 except that a heating roller of the conventional type was prepared by forming a primer layer 2 of 6 $\mu$  in thickness containing no conductive material over an electrically conductive core member 1, and further forming a PFA resin layer 3 of 30 to 40 $\mu$  in thickness over the primer layer 2. FIG. 9 shows the charging characteristics of the heating roller. The roller was negatively charged to a

maximum of -650 V after about 5 minutes passage of paper and was positively charged to a maximum of +280 V after the reversion of polarity. During the period of 2 to 5 minutes and 60 minutes after the start of passage of paper, marked offset occurred over the entire temperature range as shown in FIG. 20.

In contrast, the maximum charge potentials on the heating roller of Example 1 were inhibited to -45 V for negative polarity and +20 for positive polarity. Although there was no non-offset temperature range in the comparative example, no offset was observed in Example 1 over the temperature range of about 130° to about 220° C. during the 2-5 minute period, and over the range of about 140° to about 220° C. at the 60-minute point of time as represented by blanks in FIG. 20. In addition, there is a slight offset temperature range between the non-offset temperature range and marked offset temperature range.

The heating roller of Example 1 was further tested for long-term durability with use of 120,000 copy paper sheets. No changes were found in the anti-offset properties, while the roller was found less susceptible to defacement than the roller of the comparative example at the portions thereof in contact with the thermistor and the separating pawl. Presumably this indicates that the penetrating portions extending from the primer layer and exposed at the surface of the heating roller give improved strength to the PFA resin layer forming the surface of the heating roller.

#### EXAMPLE 2

A heat roller fixing device of the type shown in FIG. 1 was fabricated in the same manner as in Example 1 except that the heating roller was prepared with use of

0.5, 1.5 or 2.0 parts by weight of carbon black as listed in Table 1 to demonstrate the dependence of the antistatic properties of the roller on the amount of carbon added (i.e. carbon content). Generally the prevention of charging is dependent on the carbon content; the smaller the carbon content, the lower is the effect to prevent charging. However, with an excess of carbon present, the surface of the heating roller exhibits reduced release properties and consequently becomes more prone to offset. When the carbon content in Example 1 is varied to 0.5, 1.5 and 2.0 parts by weight, the heating roller exhibits the charging characteristics shown in FIGS. 11, 12 and 13, respectively. These drawings and Example 1 wherein the carbon content is 1.0 part by weight reveal that the effect to prevent charging of both positive and negative polarities increases with an increase in the carbon content. Accordingly when the carbon content is 0.5 part by weight which is less than in Example 1, the maximum charge potentials are -65 V for negative polarity and +47 V for positive polarity, thus exhibiting a tendency toward slightly greater chargeability than in Example 1. Nevertheless, the result is exceedingly superior to that achieved in the comparative example.

As to the likelihood of offset, on the other hand, FIG. 20 shows at the carbon contents of 0.5, 1.5 and 2.0 parts by weight wide non-offset temperature ranges which are comparable to the corresponding range of Example 1.

When tested for durability, the heat rollers were found to be as satisfactory as the roller of Example 1.

### EXAMPLE 3

The thickness of the PFA resin layer as the second layer influences the connection between the penetrating portions from the first layer of primer and those from the third layer of primer and consequently governs the charging characteristics of the heating roller. To investigate the dependence of the charging characteristics on the thickness of the second layer of PFA resin, a heat roller fixing device of the type shown in FIG. 1 was fabricated in the same manner as in Example 1 except that the heating roller was prepared by forming the second layer of PFA resin in a thickness of 5 $\mu$ , 15 $\mu$  or 30 $\mu$ , forming the second layer of primer in a thickness of 5 $\mu$  and thereafter removing the 5- $\mu$ -thick primer layer by grinding as listed in Table 1.

When the thickness of the PFA resin layer is 5 $\mu$ , 15 $\mu$  and 30 $\mu$ , the heating roller exhibits the charging characteristics of FIGS. 14, 15 and 16, respectively. Although the charging preventing effect slightly decreases as the thickness is reduced, the maximum charge potentials at the largest thickness of 30 $\mu$  are -12 V for negative polarity and about +5 V for positive polarity, thus showing fairly high antistatic properties. This appears to indicate that when the finely divided PFA resin of the second layer is baked, the carbon black-containing primer of the first layer and the carbon black-containing primer of the third layer sandwiching the second layer both partly penetrate into the second layer and become connected at the penetrating portions even if the second layer of PFA resin has a somewhat increased thickness.

As to the likelihood of offset at varying temperatures, FIG. 20 shows a slightly lower offset preventing effect at a high temperature range than in the case of Examples 1 and 2. In practice, however, no problem will arise since no offset occurs over the fixing temperature range actually used.

When tested for durability, the heating rollers were found to be as satisfactory as the roller of Example 1.

### EXAMPLE 4

5 A heat roller fixing device of the type shown in FIG. 1 was fabricated in the same manner as in Example 1 except that the thickness of the fourth layer of PFA resin of the heating roller was altered as listed in Table 1 to determine the dependence of prevention of charging on the thickness of the fourth layer. When the fourth layer of PFA resin is formed in a thickness of 23 $\mu$  or 30 $\mu$  and then removed by a thickness of 5 $\mu$  by grinding, the heating roller exhibits the charging characteristics shown in FIG. 17 or 18. These drawings and Example 1 wherein the fourth PFA resin layer is 15 $\mu$  in thickness indicate that the effect to prevent negative charging decreases as the thickness of the fourth layer increases, and that the rate of the decrease is greater than when the thickness of the second layer of PFA resin is increased in Example 3. Presumably this is attributable to the fact that the carbon black-containing primer of the third layer alone penetrates into the fourth PFA resin layer.

As to the offset of positively charged toner at varying temperatures, the present example and Example 1 reveal that as the thickness of the fourth layer of PFA resin increases, the marked offset temperature range, as well as the slight offset temperature range, increases to reduce the non-offset temperature range.

These results indicate that the prevention of charging of both positive and negative polarities is dependent largely on the thickness of the fourth PFA resin layer. That is, with the standard structure wherein the first layer of primer is 5- $\mu$  thick, the second layer of PFA resin is 15- $\mu$  thick and the third layer of primer is 5- $\mu$  thick, the fourth PFA resin layer should preferably be about 15 to 20 $\mu$  in thickness.

When tested for durability, the heating rollers were found to be as satisfactory as the roller of Example 1.

### EXAMPLE 5

A heat roller fixing device of the type shown in FIG. 1 was fabricated in the same manner as in Example 1 with the exception of using 1.5 parts by weight of carbon black and forming the first layer of primer in a thickness of 15 $\mu$  and the second layer of PFA resin in a thickness of 35 $\mu$ , without forming the third layer of primer and the fourth layer of PFA resin as shown in Table 1.

When the heating roller is to be fabricated in the form of a two-layer structure without forming the third layer of primer, it is generally necessary to give an increased thickness of 30 to 40 $\mu$  to the second layer of PFA resin. The present example substantiates the dependence of the prevention of charging on the thickness of the first primer layer in this case.

With reference to FIG. 19 showing the charging characteristics of the heating roller, the effect to prevent negative charging only is slightly lower than the heating roller of Example 2 shown in FIG. 12 and containing 1.5 parts by weight of carbon black but does not involve the phenomenon observed with the roller of Example 4 wherein the fourth layer of PFA resin is 30 $\mu$  in thickness (FIG. 18). This appears attributable to the increased thickness, i.e., 15 $\mu$ , of the first primer layer which accelerates the penetration of the primer into the second PFA resin layer although the second layer is as thick as 35 $\mu$ .

As to the occurrence of offset at varying temperatures, FIG. 20 reveals a wide non-offset temperature range which is comparable to those determined for Examples 1 and 2.

When tested for durability, the heating roller was found as satisfactory as the roller of Example 1.

While the present invention has been described above primarily with reference to heating rollers of four-layer structure, heating rollers of three-layer structure wherein the third layer is removed by grinding fully achieve the object of inhibiting positive and negative charging to prevent offset as apparent from Example 3. Even in the case of those originally designed to have a two-layer structure without the third layer of primer, in view of the relation of the depth of scratches or defacement due to the contact of the separating pawl or thermistor to the thickness and strength (hardness) of the PFA resin layer, similar effects can be obtained by increasing the thickness of the first primer layer as demonstrated by Example 5. Additionally, when an increased thickness is given to the third layer of primer as in Example 4, the heating roller becomes usable even if the fourth layer of PFA resin has a thickness of 30 $\mu$ .

What is claimed is:

1. A heat roller fixing device which comprises a heating roller constituted by a fluorine resin layer laminated on an electrically conductive core member through a primer layer, heating means incorporated in said core member, said heating roller being driven for rotation by driving means, and a pressure roller constituted by an electrically insulative layer on another electrically conductive core member and held in contact under pressure with said heating roller for simultaneous rotation with said heating roller, thereby fixing a charged toner image formed on copy paper onto the copy paper by causing said copy paper carrying said toner image thereon to pass between said heating roller and said pressure roller, said primer layer being composed of a primer having incorporated therein an electrically conductive material, the primer of said primer layer being partially exposed at an exposed outer surface of said fluorine resin layer.

2. A heat roller fixing device as claimed in claim 1, wherein the primer of said primer layer partially exposed at the surface of said fluorine resin layer comprises penetrating portions partially extending from said primer layer, said penetrating portions being formed in said fluorine resin layer and being very well dispersed therein.

3. A heat roller fixing device as claimed in claim 2, wherein the surface of said fluorine resin layer is electrically connected to said electrically conductive core member by said primer layer and said penetrating portions formed in said fluorine resin layer.

4. A heat roller fixing device as claimed in claim 1, wherein the electrically conductive material incorporated into said primer is carbon black.

5. A heat roller fixing device as claimed in claim 4, wherein the amount of the carbon black is 0.4 to 3.0% by weight.

6. A heat roller fixing device as claimed in claim 1, wherein the fluorine resin of said fluorine resin layer is a polytetrafluoro ethylene perfluoro alkoxy ethylene copolymer resin.

7. A heat roller fixing device which comprises a heating roller constituted by first and second fluorine resin layers and first and second primer layers formed alternately over one another on an electrically conductive core member so as to form a surface of the heating roller by said second fluorine resin layer and having heating means incorporated in said heating roller, said heating roller being driven for rotation by driving means, and a pressure roller constituted by an electrically insulative layer on another electrically conductive core member and held in contact under pressure with the heating roller for simultaneous rotation with said heating roller, thereby fixing a charged toner image formed on copy paper onto the copy paper by causing said copy paper carrying said toner image thereon to pass between said heating roller and said pressure roller, said primer layers being composed of a primer having incorporated therein an electrically conductive material, the primer of the second, upper primer layer being partially exposed at an exposed outer surface of the second, outer fluorine resin layer, and the primer of the first and second primer layers partially penetrating into the first, inner fluorine resin layer sandwiched between the two primer layers.

8. A heat roller fixing device as claimed in claim 7, wherein the primer of said upper primer layer partially exposed at the surface of said outer fluorine resin layer comprises penetrating portions partially extending from said upper primer layer, said penetrating portions being formed in said outer fluorine resin layer and being very well dispersed therein and the primer of said two primer layers being partially continued in said inner fluorine resin layer by penetrating portions partially extending from said two primer layers, said penetrating portions being formed in said inner fluorine resin layer and being very well dispersed therein.

9. A heat roller fixing device as claimed in claim 8, wherein the surface of said outer fluorine resin layer is electrically connected to said electrically conductive core member by said two primer layers and said penetrating portions formed in said two fluorine resin layers.

10. A heat roller fixing device as claimed in claim 7, wherein the electrically conductive material incorporated into said primer is carbon black.

11. A heat roller fixing device as claimed in claim 10, wherein the amount of the carbon black is 0.4 to 3.0% by weight.

12. A heat roller fixing device as claimed in claim 7, wherein the fluorine resin of said two fluorine resin layers is a polytetrafluoro ethylene perfluoro alkoxy ethylene copolymer resin.

13. A heat roller fixing device for fixing a charged toner image formed on copy paper onto the copy paper, which comprises a heating roller constituted by at least one primer layer composed of a primer having incorporated therein an electrically conductive material and at least one fluorine resin layer over said primer layer, said fluorine resin layer having formed therein penetrating portions of said primer partially extending from said primer layer.

14. A heat roller fixing device as claimed in claim 13, wherein the penetrating portions of said primer are exposed at an exposed outer surface of said fluorine resin layer.

\* \* \* \* \*